

1

2,983,598

## METHOD OF MAKING CORROSION-RESISTANT STEEL

Charles W. Wheatley, Milwaukee, Wis., assignor to A. O. Smith Corporation, Milwaukee, Wis., a corporation of New York

No Drawing. Filed Dec. 15, 1958, Ser. No. 784,831

1 Claim. (Cl. 75—56)

This invention relates to a method of making steel having an increased resistance to corrosion from an alkaline medium.

It has been found that steel having a low silicon content and a plurality of oxygen rich areas throughout the structure exhibits excellent resistance to corrosion from an alkaline medium and this resistance is particularly evident when the rolled steel contains banded layers or striations of oxides.

The present invention is directed to a method of making this specially processed steel in which the oxides are present in the rolled product in the form of striations or bands.

According to the invention the method consists of uniformly adding finely divided mill scale or other relatively impure forms of iron oxide, such as iron ore, to the steel during teeming in an amount equivalent to at least 1.75 pounds of mill scale per ton of steel and thereafter plating or capping the steel ingot to solidify the steel and terminate the reduction of the oxides by the carbon present in the steel. Terminating the reduction of the oxides results in the steel retaining a carbon content in excess of 0.12% and having substantially uniformly distributed areas of oxides throughout the ingot. The ingot is subsequently rolled into plate or wrought products and the rolling deforms the oxygen rich areas into striations or bands which offer maximum resistance to corrosive attack from an alkaline medium.

In the past, mill scale has been added in small amounts to keep the heat open and increase the amount of rim. Generally the mill scale has been added to the ladle but occasionally mill scale, in small amounts up to 0.5 pound per ton of steel, has been added to the ingot mold to keep the heat open. However, mill scale added to the ladle or added to the mold in these small amounts will not result in the oxygen rich areas which are essential to the present invention nor will it result in the oxides being present in the desired striated form. By adding the mill scale or other equivalent form of iron oxides in an amount of at least 1.75 pounds per ton during teeming and thereafter plating or capping the ingot to prevent the complete reaction between the carbon of the steel and the iron oxides can the desired oxygen content in striated oxide form be obtained.

Other objects and advantages of the present invention will appear in the course of the following description of the invention.

The corrosion-resistant steel of the present invention has the following range of chemical composition as determined by conventional ladle analysis before the addition of the iron oxides:

|                                              |                |
|----------------------------------------------|----------------|
| Carbon                                       | 0.30% maximum. |
| Manganese                                    | 1.00% maximum. |
| Silicon                                      | 0.10% maximum. |
| Total phosphorus, sulphur and trace elements | 1.00% maximum. |
| Iron                                         | Balance.       |

2

The carbon content, by ladle analysis, while maintained under 0.30%, should generally be between about 0.15% and 0.30% so that the resulting steel will have a carbon content of 0.12% to 0.27% to provide adequate mechanical properties to be utilized for structural purposes such as the fabrication of vessels or the like.

It is essential that the silicon content be maintained below 0.10% for it has been found that a silicon content above this maximum results in a considerable decrease in the corrosion resistance of the steel to alkaline attack.

To obtain the desired oxygen rich areas and striated form in the rolled product, mill scale, or other unpurified forms of iron oxide, such as iron ore, is added into the ingot mold. The mill scale which is essentially  $Fe_3O_4$ , or a combination of  $Fe_3O_4$ ,  $Fe_2O_3$  and  $FeO$ , is added during the teeming of the steel so as to produce the eventual distribution of the oxides in the steel necessary to achieve the desired resistance to alkaline corrosion of the plate steel or wrought products into which the ingot is ultimately formed.

The mill scale is added in a quantity of at least 1.75 pounds per ton of steel with a range of 2.5 to 6.0 pounds of mill scale or its equivalent per ton of steel having been found to be very satisfactory for most purposes.

The mill scale is added to the mold in a finely divided state to achieve a uniform distribution of the oxides in the steel. It has been found that discrete particles having a size of  $\frac{1}{4}$  inch or smaller will produce this desired uniform distribution. The use of larger sized particles or lumps will result in a less uniform distribution of the oxides in the steel and in extreme cases the mill scale may not go into solution in the steel but will remain as included areas of mill scale, which are objectionable.

The finely divided mill scale or equivalent form of iron oxide is added generally continuously and uniformly to the ingot mold during teeming at a rate determined by the operator and the effervescence of the metal to obtain a uniform distribution of the oxides in the metal. Generally, the operator adds the mill scale to the mold during the entire pouring operation at the maximum rate possible without causing the steel to boil up over the top of the mold. The addition of mill scale at this rate will result in the 2.5 to 6.0 pounds of mill scale per ton of steel range set forth above.

In order to produce the oxygen rich areas in the steel as well as maintaining the carbon content above 0.12% so that the steel will have adequate mechanical properties, it is essential that the mill scale be added to the ingot mold during teeming and that the mold be plated or capped to solidify the steel and minimize the reduction of the oxides by the carbon present in the steel. The addition of mill scale or the equivalent form of iron oxide to the ladle, instead of to the ingot mold, will not produce the desired properties in the steel, for a more complete reaction between the oxides and the carbon of the steel will occur, resulting in both a reduced oxide content and a decreased carbon content in the solidified steel.

In the present invention the mill scale is added to the mold during the entire pouring of the steel into the mold, and on completion of pouring, the ingot is capped or plated to terminate the reduction of the oxides by the carbon. The plating is done after a given thickness of solidified steel crust forms on the outer surface of the ingot. The thickness of steel crust is judged by the operator, and the required thickness before plating depends largely on the size of the ingot and is usually about 4 to 6 inches. Generally, the time between the completion of pouring and the plating of the ingot is from 10 to 20 minutes.

The plating or capping of the ingot serves to cool and solidify the top layer of the steel and prevents the evolu-

tion of gas from the steel. The plating in effect terminates the reaction between the oxides and the carbon of the steel and prevents complete reduction of the oxides by the carbon. This results in the steel retaining a carbon content in the range of 0.12% to 0.27% and also having uniformly distributed oxygen rich areas which appear in the desired striated form when the ingot is subsequently rolled.

After the ingot has solidified it is transferred to a soaking pit which is at a temperature of about 1800° F. to 2000° F. When the temperature of the ingot has reached equilibrium with the temperature of the soaking pit, the ingot is heated to the rolling temperature of about 2400° F. After the ingot has been heated through to the rolling temperature it is removed for rolling. Soaking or prolonged periods of heating of more than one hour at the rolling temperature results in a diffusion of the oxides which is undesirable, and thus the ingot is removed from the soaking pit shortly after being heated through.

The ingot is rolled by conventional practices normally used in the production of steel plate or wrought products, and the rolling operation tends to produce striations or banded layers having a high concentration of oxide inclusions. These banded layers are believed to consist of the oxide inclusions surrounded by areas of iron supersaturated with oxygen. The oxygen in solid solution is thought to originate from the  $Fe_3O_4$  or mill scale and diffuses into the iron during heating and rolling.

The presence of the oxide striations can be observed by microscopic examination of polished and etched metallographic samples. The steel in this sample was made in accordance with the present invention by adding 75 pounds of mill scale to a 20 ton ingot during teeming. The sample was taken from a rolled plate representative of the center portion of the ingot. The ladle analysis of the steel and the analysis of the sample are as follows in weight percent:

|             | C   | Mn  | P    | S    | Si   | Fe      |
|-------------|-----|-----|------|------|------|---------|
| Ladle.....  | .21 | .51 | .013 | .030 | .009 | Balance |
| Sample..... | .18 | .56 | .012 | .032 | .004 | Balance |

The sample was etched for 3.5 minutes in the following boiling solution established in the art to particularly reveal oxygen rich areas:

|              |       |     |
|--------------|-------|-----|
| NaOH         | grams | 30  |
| $K_2Cr_2O_7$ | do    | 4   |
| $KMnO_4$     | do    | 10  |
| $Na_2CO_3$   | do    | 10  |
| $H_2O$       | ml    | 100 |

Definite bands or striations, shown as the lighter areas in the etched sample, exist in the plate and these oxygen rich bands are disposed generally parallel to the plate surface, thereby affording the most desirable resistance to corrosive attack from alkaline media.

The banded condition of the oxides, as evidenced by the aforementioned etching procedure, can be further accentuated by thermal treatment. By heating the steel to a temperature above 1150° F. and below the lower critical temperature of the steel and maintaining the

steel at this temperature for a period of least two hours, the banded condition of the oxides can be further defined and accentuated.

The oxygen content of the plate may be determined by means of vacuum fusion in a graphite crucible. However, as the oxides in the plate are not uniformly distributed throughout the plate, but instead are concentrated as bands or striations, it is difficult to obtain an accurate determination of the oxygen content. Generally speaking, the oxygen content of the plate should be in the range of 0.005% to 0.05% with a preferred range of 0.01% to 0.03%, but as previously set forth, the banded or striated form of the oxides brought about by the aforementioned addition of mill scale is the feature which is most important in bringing out the improved corrosion resistance to the alkaline media rather than the specific oxygen content of the plate.

The present invention provides a simple and inexpensive method of producing a steel having a plurality of oxygen rich areas throughout the structure disposed in a banded form. The high oxide content and banded condition of the same, results in a steel which exhibits excellent resistance to corrosion from alkaline solutions, such as that encountered in sulphate digesting processes.

This application is a continuation-in-part of application Serial No. 482,187, filed January 17, 1955, now abandoned, and entitled Method of Making Corrosion Resistant Steel.

Various modes of carrying out the invention are contemplated as being within the scope of the following claim particularly pointing out and distinctly claiming the subject matter which is regarded as the invention.

I claim:

A method of making structural steel to be fabricated into an article subjected in service to an alkaline medium, comprising adding to the ingot mold as the steel is poured into said mold iron oxide equivalent to at least 1.75 pounds of mill scale per ton of steel and at a rate determined by the effervescence of the steel to obtain a substantially uniform distribution of the oxide throughout the ingot, said steel as poured having a carbon content in the range of 0.15% to 0.30% and said iron oxide being in the form of fine particles added substantially continuously during the entire pouring operation, capping the steel ingot within a period of time sufficient to prevent a complete reaction between the iron oxide and the carbon in the steel to maintain a carbon content in the range of 0.12% to 0.27% in the solidified steel and said solidified steel containing oxygen rich areas substantially uniformly distributed throughout the steel, and thereafter rolling the ingot to deform said oxygen rich areas into striations resistant to attack from an alkaline media when said steel is fabricated into the article.

55 References Cited in the file of this patent

| UNITED STATES PATENTS |         |               |
|-----------------------|---------|---------------|
| 92,667                | Stewart | July 13, 1869 |
| 2,181,693             | Epstein | Nov. 28, 1939 |
| 60 2,236,504          | Herty   | Apr. 1, 1941  |